

1

3,486,866

QUATERNARY AMMONIUM IODIDE STABILIZED  
FUELSVerner L. Stromberg and David B. Guthrie, St. Louis,  
Mo., assignors to Petrolite Corporation, Wilmington,  
Del., a corporation of Delaware  
No Drawing. Filed Jan. 5, 1966, Ser. No. 518,781  
Int. Cl. C10I 1/22

U.S. Cl. 44—72

6 Claims

## ABSTRACT OF THE DISCLOSURE

A distillate fuel composition comprising a major amount of distillate fuel having a distillation range between about 100° F. and about 750° F. and boiling substantially continuously throughout said distillation range and distillate fuel soluble quaternary ammonium iodide additive in a minor amount sufficient to inhibit oil deterioration with the attendant formation of color and sludge.

This invention relates to improved fuel oil compositions. More particularly, it is concerned with the provision of fuel oils which have been stabilized against the formation of color and sediment therein during storage.

Fuel oils in general are contemplated by the invention. The fuel oils with which this invention is especially concerned are hydrocarbon fractions having an initial boiling point of at least about 100° F. and an end point not higher than about 750° F., and boiling substantially continuously throughout their distillation range. Such fuel oils are generally known as distillate fuel oils. It will be understood, however, that this term is not restricted to straight-run distillate fractions. Thus, as is well known to those skilled in the art, the distillate fuel oils can be straight-run distillate fuel oils, catalytically or thermally cracked (including hydrocracked) distillate fuel oils, or mixtures of straight-run distillates, naphthas and the like, with cracked distillate stocks. Moreover, such fuel oils can be treated in accordance with well known commercial methods, such as acid or caustic treatment, solvent refining, clay treatment, etc.

The distillate fuel oils are characterized by their relatively low viscosities, low pour points, and the like. The principal property which characterizes the contemplated hydrocarbon fractions, however, is the distillation range. As mentioned herein, this range will lie between about 100° F. and about 750° F. Obviously, the distillation range of each individual fuel oil will cover a narrower range falling, nevertheless, within the above-specified limits. Likewise, each fuel oil will boil substantially continuously throughout its distillation range.

Especially contemplated herein are Nos. 1, 2 and 3 fuel oils used in domestic heating and as diesel fuel oils, particularly those made up chiefly or entirely of cracked distillate stocks. The domestic heating oils generally conform to the specifications set forth in A.S.T.M. Specifications D396-48T. Specifications for diesel fuels are defined in A.S.T.M. Specifications D975-48T. Also contemplated herein are fuels for jet combustion engines. Typical jet fuels are defined in Military Specification MIL-F-5624B.

As is well known, fuel oils have a tendency to deteriorate in storage and form soluble colored bodies and insoluble sludge therein. This deterioration of the oil is highly undesirable in that it causes serious adverse effects on the characteristics of the oil, particularly on the ignition and burning qualities thereof. It is also a contributory factor, along with the presence of other impurities in the oil, such as rust, dirt and moisture, in causing clogging of the equipment parts, such as screens, filters, noz-

2

zles, etc., as is explained further herein. An important economical factor is also involved in the problem of oil deterioration in storage, viz, customer resistance. Thus, customers judge the quality of an oil by its color and they oftentimes refuse to purchase highly colored oils. It will be appreciated then that since fuel oils of necessity are generally subject to considerable periods of storage prior to use, the provision of a practical means for preventing the deterioration of the fuel oil during storage would be a highly desirable and important contribution to the art.

The problem of the formation of color bodies and sludge is further aggravated because fuels, such as diesel and jet fuels, are often preheated for some time before consumption, thus introducing the additional problem of thermal instability.

We have now found that oil deterioration, with attendant formation of color and sludge in the oil, can be outstandingly inhibited by employing the quaternary ammonium iodide systems of this invention in the oil. In general, one employs a minor amount of the additive which is sufficient to inhibit oil deterioration with the attendant formation of color and sludge.

The amount of additive employed will vary depending on various factors, for example the particular oil to be stabilized, the conditions of storage, etc. The stability of an oil depends largely on the nature of the crude oil from which it is made, the type of processing involved during refining, etc., and therefore some oils will require more additive to stabilize them than others. For example, caustic-treated oil will, in general, require less additive than untreated oil of similar character. In practice, one generally employs at least about .0001% (1 p.p.m.), such as from about .0001 to .1% (1-1000 p.p.m.), for example about .0002 to .05% (2-500 p.p.m.), but preferably about .0003 to .03% (3-300 p.p.m.) based on weight of oil. Larger amounts, such as 1% or higher, can be employed but in general there is usually no commercial advantage in doing so.

The quaternary ammonium iodides of this invention can be prepared by any conventional means, but should be soluble in the fuel. For example, one can prepare an oil soluble quaternary ammonium iodide by the alkylation of an oil soluble tertiary amine with any alkyl, benzyl, etc., iodide; the iodide, for example, contains at least one carbon atom and may contain up to thirty carbon atoms or more per molecule. However, to convert an oil insoluble amine to an oil soluble quaternary ammonium iodide one must use an alkyl iodide of sufficient molecular weight to accomplish this. For economic reasons, it is usually preferred to start with an oil soluble tertiary amine.

The quaternary ammonium iodide systems of this invention include those derived from tertiary monoamines. A monoamine suitable for the ultimate conversion to a quaternary ammonium iodide of this invention may be defined by the formula  $R_3N$ , where the R's, which may be the same or different, are hydrocarbon or substituted hydrocarbon groups, for example, alkyl, cycloalkyl, aryl, alkenyl, substituted aryl, aralkyl, oxygen-containing, sulfur-containing, heterocyclic radical including cyclic amino wherein the nitrogen is part of the ring, etc. Each R group on the amine can vary widely, for example from 1-30 or more carbons. However, to provide the amine with sufficient hydrocarbon content to render it soluble in the fuel, the monoamines most advantageously employed are those which have a total carbon content of at least 8 atoms per molecule; and where at least one R group is as follows: hexyl, heptyl, octyl, isooctyl, t-octyl, nonyl, decyl, undecyl, dodecyl, t-dodecyl, tridecyl, tetradecyl, pentadecyl, hexadecyl, heptadecyl, octadecyl, eicosyl, docosyl, octadecenyl, octadecadienyl, octadecatrienyl, mixtures of the foregoing radicals, radicals as derived

from tallow, soybean, coconut oil and other animal and vegetable oils, and hydrocarbon radicals derived from the acids of rosin and tall oil, such as abietic acid, dehydroabietic acid and tetrahydroabietic acid, petroleum, etc.; one or more of the R's in the amine may be a lower hydrocarbon radical, for example, methyl, ethyl, propyl, butyl, pentyl, hexyl, heptyl, etc. or isomers analogues thereof etc., for example, isopropyl, isobutyl, secondary butyl, etc. An example of a quaternary ammonium iodide of this invention derived from a tertiary monoamine is:



Examples of commercially available tertiary monoamines which can be employed in the preparation of quaternary ammonium iodides of this invention are those based on fatty amines sold under the "Armeen" trademark manufactured and sold by Armour & Company of Chicago, Illinois, such as "Armeen DM12D," "Armeen DM14D," "Armeen DM16D," "Armeen DM18D," "Armeen DMCD," "Armeen DMSD," "Armeen DMHTD," "Armeen M2HT," and N-coco-morpholine. The code for these compounds is DM for dimethyl, M for methyl, CD for distilled coconut oil amine, SD for distilled soybean oil amine, 2HTD for distilled dihydrogenated tallow amine and the 12D, 14D, 16D and 18D are distilled fatty amines containing predominantly the number of carbon atoms specified in the code number.

In addition to the quaternary ammonium iodides of tertiary monoamines, other suitable systems of this invention include the product of a mixture of an alkyl iodide or aralkyl iodide with the derivatives of primary amines such as, for example, the Schiff's base or azomethine of a "Primene."



These Schiff bases or azomethine compounds are described in U.S. Patent 2,701,187 which is by reference incorporated into the present application.

Quaternary ammonium iodides of this invention also include those systems derived from tertiary monoamines which are hydroxylated monoamines. The hydroxylated monoamines employed as precursors for the quaternary ammonium iodides of this invention are monoamines containing at least one hydroxy group, usually in the form of an alkanol group ( $-\text{R}-\text{OH}$ ) and may contain as many of these groups as there are available positions in the molecule, particularly at the amino positions. Thus, they may be:



and the like, where R' is a hydrocarbon, or a substituted hydrocarbon group, for example alkenyl, alkyl, cycloalkyl, aryl, aralkyl, substituted aryl, oxygen-containing group, heterocyclic group, including the R' groups which may be joined together so as to form a heterocyclic ring with the nitrogen, and the like; and where R is a hydrocarbon group, for example,  $(\text{CH}_2)_x$  (where x is a whole number, preferably 2-8),



and other members of the homologous series. Thus, any primary or secondary amine may be oxyalkylated to form dihydroxy tertiary amines or monohydroxy tertiary amines, respectively.

The quaternary ammonium iodide systems of this invention contain at least one quaternary ammonium group and are represented symbolically, for convenience, as:



where



10 represents a quaternary ammonium moiety. These include mono-, di- and polyquaternaries. Not all of the amino groups in the molecule need to be quaternized. A more specific formula can be expressed by the general formula:



where N represents the quaternary ammonium nitrogen atom; R<sub>1</sub>, R<sub>2</sub>, R<sub>3</sub>, R<sub>4</sub> may be alkyl, aryl, aralkyl, cycloalkyl, alkenyl, substituted aryl, oxygen-containing groups, nitrogen-containing groups, sulfur-containing groups, heterocyclic groups, etc. The R's may be the same or different. Two of the R groups may be joined together so as to form a nitrogen containing ring.

A preferred class of commercial monoamines that can be hydroxylated to a suitable precursor amine for conversion to quaternary ammonium iodides of this invention are those sold under the trademark "Primene" by Rohm & Hass, which are described in their Technical Bulletin SP-33, dated December 1951 and in their other bulletins. A "Primene" is a tertiary alkyl primary monoamine which is characterized by the terminal structural unit.



It may also be expressed by the formula



where n is for example 0-5.

45 Specific tertiary alkyl primary monoamines for preparing suitable precursor amines for conversion to quaternary ammonium iodides contemplated by the invention are, for example: tertiary butyl primary amine, tertiary octyl primary amine, tertiary decyl primary amine, tertiary dodecyl primary amine, tertiary tetradecyl primary amine, tertiary hexadecyl primary amine, tertiary octadecyl primary amine, tertiary eicosyl primary amine, tertiary docosyl primary amine and tertiary tetracosyl primary amine, and mixtures of tertiary alkyl primary amines having 55 from about 4 to about 24 carbon atoms; a typical mixture of amines, for example, is one comprised of tertiary alkyl primary amines of from about 12 to 15 carbon atoms, said mixture averaging about 12 carbon atoms per amine molecule. This mixture, designated hereinafter as "mixture A," 60 contains, by weight, about 85% of tertiary dodecyl amine, about 10% of tertiary pentadecyl amine and relatively small amounts, i.e., less than about 5% of amines having less than 12 or more than 15 carbon atoms. Another mixture of tertiary alkyl primary amines is composed of 65 tertiary alkyl primary amines of from about 18 to 24 carbon atoms and averaging about 20 carbon atoms per molecule. This latter mixture, designated hereinafter as "mixture B," contains the C<sub>18</sub>-C<sub>24</sub> tertiary alkyl primary amines in about the following proportions:

|                               | Percent |
|-------------------------------|---------|
| Tertiary octadecyl amine      | 40      |
| Tertiary eicosyl amine        | 30      |
| Tertiary docosyl amine        | 15      |
| Tertiary tetracosyl amine     | 10      |
| 75 Other amines and non-amine | 5       |

Amine mixtures, such as "mixture A" and "mixture B," as well as other suitable mixtures of tertiary alkyl primary amines of 4 to 24 carbon atoms, can be prepared by methods within the knowledge of those skilled in the art. For example, such mixtures may be prepared from polypropylene or polybutylene fractions or mixtures thereof. Thus, a selected polymer fraction composed of mixed polyolefins within a desired molecular weight range can be converted to the corresponding tertiary alkyl primary amines as follows: The selected polyolefin fraction is first hydrated by means of sulfuric acid and water to convert it to the corresponding alcohols. The alcohol mixture is then converted to alkyl chlorides by reaction with dry hydrogen chloride. Finally, the alkyl chloride mixture is condensed under pressure with ammonia to produce the tertiary alkyl primary amine mixture. Specific methods of preparing the tertiary alkyl primary amines are disclosed in the Journal of Organic Chemistry, vol. 20 (1955), page 295 et seq.

The "Primene" type primary monoamine may be readily converted to a tertiary hydroxylated monoamine by reaction with alkylene oxide and alkylation as necessary. This type of suitable precursor amine now contains another functional group (the hydroxy group) besides the amino group. Thus, for example, a  $N,N$ -bis(hydroxyalkyl) tertiary alkyl mono-amine and  $N$ -alkyl- $N$ -(hydroxyalkyl) tertiary alkyl monoamine, such as,  $N,N$ -bis(2-hydroxyethyl) tertiary octyl amine and  $N$ -ethyl- $N$ -(2-hydroxyethyl) tertiary octyl amine and  $N$ -methyl- $N$ -(2-hydroxyethyl) tertiary octyl amine, respectively, can be used for subsequent conversion to a quaternary ammonium iodide.

The hydroxylated monoamines so described can be treated with additional alkylene oxide, for example, ethylene oxide, propylene oxide, butylene oxide, octylene oxide and other aliphatic oxides, glycide as well as aromatic oxides such as styrene oxide and similar compounds to form hydroxylated amines having repetitive ether linkages. Such resulting hydroxylated amines may be described by the formula



wherein, X, Y and Z are either hydrocarbon groups or  $(RO)_zH$  groups (where z is a whole number, for example 1-10 or higher and where R is the hydrocarbon moiety derived from the alkylene oxide).

These monoamines contain at least one hydroxyl group, but may have two or three or even more. For example, a tertiary amine compound having four hydroxyl radicals can be prepared from a primary amine such as octylamine, dodecylamine, octadecylamine or the like by reaction with two moles of glycide. Similarly, if a mole of triethanol, tripropanol or tributanol amine is reacted with three moles of glycide, one obtains a monoamine having as many as six hydroxyl radicals. In addition, one or more of the terminal OH groups in the molecule may be blocked by an ether or an ester linkage, for example, as in compounds of the type:



Quaternary ammonium iodides of this invention also include those derived from hydroxylated polyamines and non-hydroxylated polyamines which contain at least one tertiary amine. A wide variety of polyamines can be employed as long as there is at least one tertiary amino group which is capable of forming the quaternary ammonium group. The polyamines prior to their formation as tertiary polyamines include aliphatic polyamines, cycloaliphatic polyamines, aromatic polyamines, heterocyclic polyamines and polyamines containing one or more of the above groups. Thus, the term "polyamine" includes

compounds having one amino group on one kind of radical, for example, an aliphatic radical, and another amino group as the heterocyclic radical as in the case of the following formulae:



It also includes compounds which are totally heterocyclic. It also includes polyamines having other elements besides carbon, hydrogen and nitrogen, for example, those also containing oxygen, etc. The preferred embodiments of the polyamines are the alkylene polyamines, the hydroxylated alkylene polyamines and the cyclic amines, and most preferably  $N$ -alkylated alkylene polyamines, for example



Polyamines are available commercially and can be prepared by well-known methods. It is well-known that olefin dichlorides, particularly those containing from 2 to 10 carbon atoms, can be converted to alkylene polyamines by reaction with ammonia or amines such as ethylamine, propylamine, butylamine, octylamine, decylamine, cetylamine, dodecylamine, etc. Cycloaliphatic and aromatic amines are also reactive. Similarly, the reaction also involves the comparable secondary amines, in which various alkyl radicals previously mentioned appear twice and are types in which two dissimilar radicals appear, for instance, amyl butylamine, hexyl octylamine, etc. If, instead of using ethylene dichloride, the corresponding propylene, butylene, amylene or higher molecular weight dichlorides are used, one then obtains the comparable homologues. One can also use alpha-omega dialkyl ethers such as  $C_1CH_2OCH_2Cl$ ,  $C_1CH_2CH_2OCH_2CH_2Cl$ , and the like. Furthermore, compounds derived by reactions involving alkylene dichlorides and a mixture of ammonia and amines or a mixture of two different amines are useful.

In using such polyalkylene polyamines it is preferred to use the polyethylene-polyamines, because of their greater commercial availability. These compounds have the formula:



wherein x is an integer varying between about two and about six.

In naming the polyalkylenepolyamine reactants, the nitrogen atoms are considered to be attached to the terminal carbon atoms of the main carbon atom chain indicated in each compound name. For example, di-(1-methylamylene) triamine has the structural formula



In numbering the main carbon atom chain, the carbon atom attached to a terminal  $-NH_2$  radical is designated as the carbon atom in the 1-position. Similar alkylene groups recur throughout the molecule. Non-limiting examples of the polyalkylenepolyamine reactants are

diethylenetriamine;

triethylenetetramine;

tetraethylenepentamine;

di-(methylether) triamine;

hexapropylene-heptamine;

tri(ethylethylene) tetramine;

penta-(1-methylpropylene)-hexamine;

tetrabutylenepentamine;  
hexa-(1,1-dimethylethylene) heptamine;  
di-(1-methylbutylene) triamine;  
pentamylenehexamine;  
tri(1,2,2-trimethylethylene) tetramine;  
di-(1-methylamylene) triamine;  
tetra-(1,3-dimethylpropylene) pentamine;  
penta(1,5-dimethamylene)-hexamine;  
di-(1-methyl-4-ethylbutylene) triamine;  
penta-(1,2-dimethyl-1-isopropylethylene) hexamine;  
tetraoctylenepentamine;  
tri-(1,4-diethylbutylene) tetramine;  
tridecylenetetramine;  
tetra-(1,4-dipropylbutylene) pentamine;  
didodecylenetriamine;  
tetradecylenepentamine;  
penta(1-methyl-4-nonylbutylene) hexamine;  
tri-(1,15-dimethylpentadecylene) tetramine;  
trioctadecylenetetramine;  
dieicosylenetriamine;  
di-(1,2-dimethyl-14-nonyltetradecylene) triamine;  
di-(1,18-dioctyloctadecylene) triamine;  
penta-(1-methyl-2-benzylethylene) hexamine;  
tetra-(1-methyl-3-benzylpropylene) pentamine;  
tri-(1-methyl-1-phenyl-3-propyl-propylene) tetramine;  
and tetra-(1-ethyl-2-benzylethylene) pentamine.

Cyclic aliphatic polyamines such as piperazine, etc. can also be employed.

Polyamines of Armour's "Duomeen" type may be employed, for example of the formula



such as



The above polyamines modified with higher molecular weight aliphatic groups, for example, those having from 8-30 or more carbon atoms, a typical example of which is



where the aliphatic group is derived from any suitable source, for example, from compounds of animal, vegetable, petroleum, etc., origin, such as coconut oil, tallow, tall oil, soya, etc., are very useful as starting materials. In addition, the polyamine can contain other alkylene groups, fewer amino groups, additional higher aliphatic groups, etc. Compositions of this type are described in U.S. Patent 2,267,205.

Polyamines containing aromatic groups in the main part of the chain, for example, N,N'-dimethyl-p-xylylenediamine, are useful as starting materials.

In order to use many of the above alkylene polyamines in the invention, the alkylene polyamines must be converted as necessary to a product containing at least one tertiary amino group for subsequent conversion to quaternary ammonium iodides. The desired tertiary polyamine can be characterized by the general formula:



where the R's, which are the same or different, comprise hydrogen, alkyl, cycloalkyl, aryl, alkoxyalkyl, hydroxylated alkyl, hydroxylated alkoxyalkyl, etc., radicals in such a combination that at least one tertiary nitrogen is possible; x is zero or a whole number of at least one, for example 1 to 10, but preferably 1 to 3; and n is a whole number, 2 or greater, for example 2-10, but preferably 2-5. Of course, it should be realized that the amino or hydroxyl group may be modified by acylation to form amides, esters or mixtures thereof.

Suitable tertiary polyamines also include tertiary polyamines wherein the alkylene group or groups are interrupted by an oxygen radical, for example,



or mixtures of these groups and alkylene groups, for example,



where R, n and x has the meaning previously stated for the linear polyamine. Polyamines may be converted to tertiary amines by any suitable introduction of hydroxylated groups. One can use any one of a number of well-known procedures such as alkylation, involving a chlorohydrin, such as ethylene chlorohydrin, glycerol chlorohydrin or the like. Such reactions are entirely comparable to the alkylation reaction involving alkyl chlorides to be subsequently described. Other reactions involve the use of an alkylene oxide, such as ethylene oxide, propylene oxide, butylene oxide, octylene oxide, styrene oxide or the like. Glycide is advantageously employed. The type of reaction just referred to is well known and results in the introduction of a hydroxylated or polyhydroxylated radical in an amino hydrogen position. It is also possible to introduce a hydroxylated oxyhydrocarbon atom; for instance, instead of using the chlorohydrin corresponding to ethylene glycol, one employs the chlorohydrin corresponding to the diethylene glycol. Similarly, instead of using the chlorohydrin corresponding to glycerol, one employs the chlorohydrin corresponding to diglycerol.

Polyalkylene polyamines having the general formula  $\text{H}_2\text{N}(-\text{RNH})_x\text{H}$  (wherein R is an alkylene radical or a hydrocarbon radical-substituted alkylene radical, and x is an integer, there being no upper limit to the number of alkylene groups in the molecule) can be alkylated with any alkyl halide which contains at least one carbon atom and up to about thirty carbon atoms or more per molecule.

Such polyamines can be alkylated in the manner commonly employed for alkylating monoamines. Such alkylation results in products which are symmetrically or non-symmetrically alkylated. The symmetrically alkylated polyamines are most readily obtainable. For instance, alkylated products can be derived by reaction between alkyl chlorides, such as propyl chloride, butyl chloride, amyl chloride, cetyl chloride, and the like and a polyamine having one or more primary amino groups. Such reaction results in the formation of hydrochloric acid, and hence the resultant product is an amine hydrochloride. The conventional method for conversion into the base is to treat with dilute caustic solution. Alkylation is not limited to the introduction of an alkyl group, but as a matter of fact, the radical introduced can be characterized by a carbon atom chain which is interrupted at least once by an oxygen atom. In other words, alkylation is accomplished by compounds which are essentially alkoxyalkyl chlorides, as, for example, the following:



It is especially preferred to use alkyl halides having between about eight and about eighteen carbon atoms per molecule. Those having between about twelve and about eighteen carbon atoms are more particularly preferred. The halogen portion of the alkyl halide reactant molecule can be any halogen atom, i.e., chlorine, bromine, fluorine and iodine. In practice, the alkyl bromides and chlorides are used, due to their greater commercial availability. Some non-limiting examples of the alkyl

halide reactant are n-butyl bromide; n-butyl chloride; sec-butyl iodide; t-butyl fluoride; n-amyl bromide; isoamyl chloride; n-hexyl bromide; n-hexyl iodide; heptyl fluoride; 2-ethyl-hexyl chloride; n-octyl bromide; decyl iodide; dodecyl bromide; 7-ethyl-2-methyl-undecyl iodide; tetradecyl bromide; hexadecyl bromide; hexadecyl fluoride; heptadecyl chloride; octadecyl bromide; docosyl chloride; tetracosyl iodide; hexacosyl bromide; octacosyl chloride and triacontyl chloride.

The alkyl halides can be chemically pure compounds or of commercial purity. Mixtures of alkyl halides, having carbon chain lengths falling within the range specified hereinbefore, can also be used. Examples of such mixtures are mono-chlorinated wax and mono-chlorinated kerosene. Methods for the preparation of mono-chlorinated wax have been set forth in United States Patent 2,238,790.

The quaternary ammonium iodides of this invention, also, include those derived from cyclic amidines which may be converted directly into quaternary ammonium iodides by reaction with alkyl iodides and aralkyl iodides. Suitable cyclic amidines include the following:



wherein R is a hydrocarbon group,



where  $x=1-5$ .

2-undecylimidazoline  
2-heptadecylimidazoline  
2-oleylimidazoline  
1-N-decylaminoethyl, 2-ethylimidazoline  
1-hexadecylaminoethylaminoethyl, 2-methylimidazoline  
1-dodecylaminopropylimidazoline  
1-(stearoyloxyethyl)aminoethylimidazoline  
1-stearamidoethylaminoethylimidazoline  
2-heptadecyl, 4-5-dimethylimidazoline  
1-dodecylaminohexylimidazoline  
1-stearoyloxyethylaminohexylimidazoline  
1-methylaminoethyl, 2-heptadecyl tetrahydropyrimidine  
1-methylaminoethylaminoethyl, 2-dodecyl, 4-methyl tetrahydropyrimidine.

Cyclic amidines such as imidazoline and tetrahydropyrimidine are well known. See U.S. Patents, 2,466,517, 2,488,163, Re. 23,227 which are by reference incorporated into the present application.

Polymeric amines can also be employed in this invention. Examples of this invention include those disclosed in the Ser. No. 442,793, filed Mar. 25, 1965; Ser. No. 502,447, filed on Oct. 22, 1965 (Docket #5-32); and Ser. No. 502,636 filed on Oct. 22, 1965 (Docket #5-16), all assigned to the same assignee as the present invention.

It should also be realized in the preparation of the cyclic amidine compounds that amides as well as cyclic amidines may be formed. By controlling the reaction of the carboxylic acids with polyamines so that one rather than two moles of water are removed, one obtains amides rather than cyclic amidines. Examples of amidopolyamines are shown in U.S. Patent 2,598,213.

The preferred system of this invention is a quaternary ammonium iodide system such as a bis oxyalkylated "Primene," or a polyoxyalkylated polyamine.

The particular amine employed can vary widely provided the derived quaternary ammonium iodide system is sufficiently soluble in the fuel to perform its function in the concentrations employed. Certain quaternary ammonium iodides which may be insoluble or only slightly soluble in the fuel when employed alone, may be rendered soluble by being employed in conjunction with other amines and/or quaternary ammonium iodide systems. Stated another way, it is not the individual quaternary ammonium iodide, but the total quaternary ammonium iodide system whose solubility must be determined.

As is quite evident, new quaternary ammonium iodides will be constantly developed which could be useful in this invention. It is, therefore, not only impossible to attempt a comprehensive catalogue of such compositions, but to attempt to describe the invention in its broader aspects in terms of specific chemical names of its components used would be too voluminous and unnecessary since one skilled in the art could by following the description of the invention herein select a useful agent. This invention lies in the use of suitable quaternary ammonium iodides as stabilizers for petroleum distillates, and the individual compositions are important only in the sense that their properties can affect its function. To precisely define each specific useful quaternary ammonium iodide in light of the present disclosure would merely call for chemical knowledge within the skill of the art in a manner analogous to a mechanical engineer who prescribes in the construction of a machine the proper materials and the proper dimensions thereof. From the description in this specification and with the knowledge of a chemist, one will know or deduce with confidence the applicability of specific quaternary ammonium iodides suitable for this invention by applying them in the process set forth herein. In analogy to the case of a machine, wherein the use of certain materials of construction or dimensions of parts would lead to no practical useful result, various materials will be rejected as inapplicable where others would be operative. One can obviously assume that no one will wish to employ a useless quaternary ammonium iodide nor will be misled because it is possible to misapply the teachings of the present disclosure to do so. Thus, any quaternary ammonium iodide that can perform the function stated herein can be employed.

The following diesel fuel test is a standard test for diesel fuel stability and is regarded as a rapid screening test for discovering new systems which can be used to stabilize petroleum distillate fuels.

In the operation of a diesel engine, a portion of the fuel sent to the fuel injection system is injected and

burned; the remainder is circulated back to the fuel reservoir. The injection system is located on the engine such that the fuel being returned to the reservoir is subjected to high temperatures. Consequently, diesel fuels should exhibit good thermal stability as well as good storage stability. Since the fuels used as diesel fuel are interchangeable with furnace oils, the following procedure is used to screen the thermal stability of fuel oils in general.

The test involves exposing 50 ml. samples of fuel, containing desired quantities of fuel additives, to the test where a bath is held at 300° F. and the samples are exposed for 90 minutes.

After cooling to room temperature the exposed fuel is passed through a moderately retentive filter paper and the degree of stain on the filter paper noted. The filter paper pads are compared according to a rating of "0, +, ++ or +++" where "0" is the amount of insoluble matter collected from the oil containing no additive, "+" is good stability and indicates a reduction in the formation of insoluble matter, "++" is superior stability and indicates a substantial reduction in the formation of insoluble matter and "+++" is excellent stability and indicates essentially no formation of insoluble matter.

In the following examples, the fuel employed was a South Central U.S. Oil containing 70% light cycle oil and 30% range oil. The following quaternary ammonium iodides were tested for their ability to stabilize fuel oil in the diesel fuel test. They are presented as examples to illustrate (rather than limit) the applicability of the invention.

| Additive: | Composition as reaction product of—                                                                |
|-----------|----------------------------------------------------------------------------------------------------|
| A         | 2 moles $\text{CH}_3\text{I} + \text{ethoduomeen}$ T/13.                                           |
| B         | 1 mole $\text{CH}_3\text{I} + \text{ethoduomeen}$ T/15.                                            |
| C         | 2 moles $\text{CH}_3\text{I} + \text{ethoduomeen}$ T/12.                                           |
| D         | 1 mole $\text{CH}_3\text{I} - \text{ethoduomeen}$ T/20.                                            |
| E         | 2 moles $\text{CH}_3\text{I} + \text{ethoduomeen}$ T/15.                                           |
| F         | 2 moles $\text{CH}_3\text{I} - \text{ethoduomeen}$ T/25.                                           |
| G         | 1 mole $\text{CH}_3\text{I} + \text{N}-(\gamma\text{-dilaurylaminopropyl})\text{morpholine}$ .     |
| H         | 2 moles $\text{CH}_3\text{I} + \text{N}-(\text{methyl-cocoamino})\text{propyl}\text{morpholine}$ . |

Ethoduomeens are commercial diamines derived from fatty amines and are available from Armour and Company. They have the general formula:



T is a code for the R-N group and is a designation for tallow amine. The numbers 12, 13, 15, 20 and 25 is a code for moles of ethylene oxide and represent the 2, 3, 5, 10 and 15 moles of ethylene oxide which were used to oxy-alkylate the tallow diamine. In other words, the numbers (12, 13, 15, 20 and 25) represent 10 more than the sum of  $x+y+z$ .

The data in Table 1 shows that excellent stability was achieved in the 90-minute 300° F. diesel fuel test.

TABLE 1—DIESEL FUEL TEST RESULTS  
 [After 90 minutes at 300° F.]  
 [Oil = Texas light cycle oil]

| Additive  | Total wt.<br>(p.p.m.) | Wt. of iodine<br>(p.p.m.) | Results after<br>heating filter<br>pad rating |
|-----------|-----------------------|---------------------------|-----------------------------------------------|
| None----- | 0                     | 0                         | 0                                             |
| A -----   | 13                    | 4.3                       | +++                                           |
| B -----   | 14.4                  | 2.6                       | +++                                           |
| C -----   | 12.4                  | 4.33                      | <+++                                          |
| D -----   | 16.7                  | 2.3                       | ++                                            |
| E -----   | 14.4                  | 4.3                       | ++                                            |
| F -----   | 20.2                  | 4.0                       | ++                                            |
| G -----   | 11.8                  | 2.4                       | ++                                            |
| H -----   | 6.8                   | 2.83                      | <++                                           |

Although quaternary ammonium iodides are useful as fuel additives, their performance can be enhanced by em-

ploying certain auxiliary chemical aids. Among these chemical aids are dispersants, for example acrylic polymers or copolymers which can be employed in conjunction with the quaternary ammonium iodide systems of this invention.

5 One such auxiliary chemical component is the copolymer derived from an acrylic ester of the formula:



and N-vinyl-2-pyrrolidone, for example, a copolymer containing the following units:



having a molecular weight for example of at least 50,000, for example 50,000-500,000, or higher, but preferably 100,000-400,000 with an optimum of 300,000-400,000 of which vinyl pyrrolidone comprises at least 1% by weight, of the polymer, for example 1-30%, but preferably 3-15% with an optimum of 5-10%; where Y is hydrogen, a lower alkyl group such as methyl, ethyl, etc., Z is an hydrocarbon group having, for example, 1-30 carbon atoms, but preferably 8 to 18 carbon atoms. These polymers are preferably acrylic or methacrylic polymers, or polymers derived from both in conjunction with vinyl pyrrolidone. The Z group on the polymer, which can be the same throughout or mixed, can be octyl, nonyl, decyl, undecyl, dodecyl, tridecyl, tetradecyl, pentadecyl, octadecyl, etc. Lower alkyl groups can also be employed such as methyl, ethyl, propyl, butyl, pentyl, hexyl, heptyl, etc., but they preferably are employed as copolymers of the higher Z groups, for example a copolymer of dodecyl methacrylate and methyl acrylate, etc. The acrylic ester units may be derived from one or more acrylic type monomers and may be fully acrylic or fully methacrylic or both acrylic and methacrylic. The polymer may be random block graft etc.

50 Also, Z may also be an alkylated aromatic group such as butyl phenyl, amyl phenyl, etc., or a cycloaliphatic group such as cyclohexyl. Thus, non-limiting specific examples of suitable monomeric esters are: methyl acrylate, ethyl acrylate, propyl methacrylate, amyl acrylate, lauryl acrylate, cetyl acrylate, octadecyl acrylate, amyl methacrylate, lauryl methacrylate, cetyl methacrylate, octadecyl methacrylate, amylphenyl methacrylate, cyclohexyl methacrylate, etc., including the analogous acrylate or methacrylate esters. Copolymers of the above and other acrylic esters may be used, for example, a copolymer of methyl or ethyl acrylate and dodecyl methacrylate in conjunction with vinyl pyrrolidone. However, it should be understood that this description does not preclude the presence of small amounts of unesterified groups being present in the polymer, i.e. approximately 5% or less of where  $Z=H$ .

It should be understood, of course, that when the above compounds are polymerized, the polymerization should not be carried to such an extent as to form polymers which are insoluble or non-dispersible in the petroleum hydro-carbon used. The polymerization may be carried out by methods known to the art, such as by heating mildly in the presence of a small amount of benzoyl peroxide, but the method of polymerization is not part of this invention. For examples of acrylic-vinyl pyrrolidone copolymers see French Patent 1,163,033.

Examples of vinyl pyrrolidone-acrylic ester type resins are presented in Table II.

4-hydroxyquinoline-aldehyde-3  
7-hydroxyquinoline-aldehyde-8

TABLE II.—VINYL PYRROLIDONE-ACRYLIC ESTER TYPE RESINS

| Example | Monomer 1              | Monomer 2              | Monomer 3          | Vinyl pyrrolidone, percent by wt. | Mol ratio 1:2:3 | Av. mol weight |
|---------|------------------------|------------------------|--------------------|-----------------------------------|-----------------|----------------|
| 1       | Tridecyl methacrylate  | Octadecyl methacrylate |                    | 7.5                               | 1:1             | 300,000        |
| 2       | Dodecyl methacrylate   |                        |                    | 10                                |                 |                |
| 3       | Dodecyl methacrylate   | Butyl acrylate         |                    | 15                                | 2:1             | 400,000        |
| 4       | Octadecyl methacrylate |                        |                    | 5                                 |                 | 450,000        |
| 5       | Tridecyl methacrylate  |                        |                    | 20                                |                 | 350,000        |
| 6       | Octadecyl methacrylate | Methyl methacrylate    |                    | 10                                | 3:1             | 500,000        |
| 7       | Dodecyl methacrylate   | Ethyl acrylate         |                    | 5                                 | 4:1             | 400,000        |
| 8       | Cetyl methacrylate     | Octadecyl methacrylate | Butyl methacrylate | 7.5                               | 2:1:0.5         | 350,000        |

Another auxiliary chemical component is a metal deactivator for example those conveniently employed in deactivating copper, iron and other metals from hydrocarbon systems. Typical examples are those described in U.S. Patent 2,282,513. Of course, one skilled in the art is aware that many other metal deactivators are known and can be employed.

The compounds employed as metal deactivators are preferably of the type of Schiff bases and may be represented by the formulae



and preferably,



wherein A and B each represents an organic radical and preferably a hydrocarbon radical. In Formula 2 A and B each preferably represents an aromatic ring or an unsaturated heterocyclic ring in which the hydroxyl radical is attached directly to a ring carbon atom ortho to the  $-\text{CH}=\text{N}$ -group. R represents an aliphatic radical having the two N atoms attached directly to different carbon atoms of the same open chain.

Typical examples of aldehyde and polyamines employed in preparing these Schiff bases include the following:

#### ALDEHYDES

Benzaldehyde  
2-methylbenzaldehyde  
3-methylbenzaldehyde  
4-methylbenzaldehyde  
2-methoxybenzaldehyde  
4-methoxybenzaldehyde  
2-naphthaldehyde  
1-naphthaldehyde  
4-phenylbenzaldehyde  
Propionaldehyde  
n-Butyraldehyde  
Heptaldehyde  
Aldol  
2-hydroxybenzaldehyde  
2-hydroxy-6-methylbenzaldehyde  
2-hydroxy-3-methoxybenzaldehyde  
2,4-dihydroxybenzaldehyde  
2,6-dihydroxybenzaldehyde  
2-hydroxynaphthaldehyde-1  
1-hydroxynaphthaldehyde-2  
Anthrol-2-aldehyde-1  
2-hydroxyfluorene-aldehyde-1  
4-hydroxydiphenyl-aldehyde-3  
3-hydroxyphenanthrene-aldehyde-4  
1,3-dihydroxy-2,4-dialdehyde-benzene  
2-hydroxy-5-chlorobenzaldehyde  
2-hydroxy-3,5-dibromobenzaldehyde  
2-hydroxy-3-nitrobenzaldehyde  
2-hydroxy-3-cyanobenzaldehyde  
2-hydroxy-3-carboxybenzaldehyde  
4-hydroxypyridine-aldehyde-3

#### POLYAMINES

Ethylenediamine  
1,2-propylenediamine  
1,3-propylenediamine  
1,6-hexamethylenediamine  
1,10-decamethylenediamine  
Diethylenetriamine  
Triethylenetetramine  
Pentaerythritoltetramine  
1,2-diaminocyclohexane  
Di-(b-aminoethyl)ether  
Di-(b-aminoethyl)sulfide

The ratio of the quaternary ammonium iodide to the metal deactivator can vary widely depending on the particular system, the fuel, etc. employed. Thus, the weight ratio of quaternary ammonium iodide to metal deactivator may be from about 0.1 to 20 or more, such as from about 8-15, but preferably from about 10-12.

The weight ratio of the quarternary ammonium iodide to the acrylic type polymer can also vary widely from about 0.1-20 or more, such as from 8-15, but preferably from about 10-12.

Having thus described our invention and what we claim as new and desire to obtain by Letters Patent is:

1. A distillate fuel composition comprising a major amount of distillate fuel having a distillation range between about 100° F. and about 750° F. and boiling substantially continuously throughout said distillation range and a minor amount, sufficient to improve stability of said fuel during storage, of distillate fuel soluble quaternary ammonium iodide additive selected from the group consisting of

- (1) N,N - bis(2 - hydroxyethyl)tertiary - octylamine iodide,
- (2) N - ethyl - N-(2-hydroxyethyl)tertiary-octylamine iodide,
- (3) N - methyl-N-(2-hydroxyethyl)tertiary-octylamine iodide,
- (4) N,N - bis(2 - hydroxyethyl)tertiary-dodecylamine iodide,
- (5) N - ethyl - N - (2-hydroxyethyl)tertiary-dodecylamine iodide,
- (6) N - methyl - N - (2-hydroxyethyl)tertiary-dodecylamine iodide,
- (7) an oxyalkylated diamine iodide of the formula



- where the sum of x, y and z is 2-15,
- (8) an oxyalkylated diamine iodide of the formula
- $$\left( \text{Tallow}-\text{N} \left| \text{CH}_2\text{CH}_2\text{CH}_2-\text{N}-\text{(CH}_2\text{CH}_2\text{O})_x \right. \right)^\oplus \text{I}^\ominus$$
- where the sum of x, y and z is 2-15,
- (9) N-( $\gamma$ -dilaurylaminopropyl)morpholine iodide, and
  - (10) N-(methyl-cocoaminopropyl)morpholine iodide.

2. The distillate fuel composition of claim 1 wherein the quaternary ammonium iodide additive is N,N-bis(2-hydroxyethyl)tertiary-dodecylamine iodide.

3. The distillate fuel composition of claim 1 wherein the quaternary ammonium iodide additive is



4. The distillate fuel composition of claim 1 wherein the quaternary ammonium iodide additive is an oxyalkylated diamine iodide of the formula



where the sum of x, y and z is 2-15.

5. The distillate fuel composition of claim 1 wherein the quaternary ammonium iodide additive is N-( $\gamma$ -dilaurylaminopropyl)morpholine iodide.

6. The distillate fuel composition of claim 1 wherein the quaternary ammonium iodide additive is N-(methylcocoaminopropyl)morpholine iodide.

#### References Cited

#### UNITED STATES PATENTS

|           |        |              |        |
|-----------|--------|--------------|--------|
| 2,321,517 | 6/1943 | Rosen        | 252-51 |
| 3,102,797 | 9/1963 | Udelhofen    | 44-72  |
| 3,317,291 | 5/1967 | Marsh et al. | 44-72  |

DANIEL E. WYMAN, Primary Examiner

Y. H. SMITH, Assistant Examiner

UNITED STATES PATENT OFFICE  
CERTIFICATE OF CORRECTION

Patent No. 3,486,866

Dated December 30, 1969

Inventor(s) Verner L. Stromberg and David B. Guthrie

It is certified that error appears in the above-identified patent and that said Letters Patent are hereby corrected as shown below:

Column 14, line 49, after "additive", there should be inserted --derived from an alkyl iodide, the alkyl having 1 to 30 carbon atoms, and a tertiary amine or a ditertiary diamine--; column 14, line 52, delete "iodide"; column 14, line 54, delete "iodide"; column 14, line 56, delete "iodide"; column 14, line 58, delete "iodide"; column 14, line 60, delete "iodide"; column 14, line 62, delete "iodide"; column 14, line 63, delete "iodide"; column 14, the formula after line 63 should read



column 14, delete lines 69-73, inclusive; column 14, line 74, "(9)" should read --(8)-- and delete "iodide"; column 14, line 75, "(10)" should read --(9)-- and delete "iodide".

Column 15, line 3, "amine" should read --alkyl ammonium--; column 15, the formula after line 5 should read



UNITED STATES PATENT OFFICE  
CERTIFICATE OF CORRECTION

Patent No. 3,486,866 Dated December 30, 1969

Inventor(s) Verner L. Stromberg and David B. Guthrie PAGE - 2

It is certified that error appears in the above-identified patent and that said Letters Patent are hereby corrected as shown below:

column 15, lines 10 and 11, delete "an oxyalkylated diamine iodide of the formula" and the formula directly thereafter should read



Column 16, line 2, "is" should read --is alkyl--; column 16, line 3, "morphopholine" should read --morpholinium--; column 16, line 5, "is" should read --is alkyl--; column 16, line 6, "morpholine" should read --morpholinium--.

SIGNED AND  
SEALED  
MAY 9 1971

(SEAL)

Attest:

Edward M. Fletcher, Jr.

Attesting Officer

WILLIAM E. SCHUYLER, JR.  
Commissioner of Patents